

# United States Patent Office

3,691,077

1

3 691 077

**3,091,077**  
**LUBRICANT COMPOSITION**

**LUBRICANT COMPOSITION**  
Robert Earl Wann, 3933 Thimblegen Drive 45239;  
Denzel Allan Nicholson, Miami Valley Lab., P.O. Box  
39175 45239; and Ted Joe Logan, Ivorydale Tech-  
nical Center 45217, all of Cincinnati, Ohio  
No Drawing. Original application Sept. 26, 1968, Ser. No.  
762,966. Divided and this application Mar. 10, 1971,  
Ser. No. 123,091

Int. Cl. C10m 1/30

U.S. CL. 252—54.6

## 6 Claims

## ABSTRACT OF THE DISCLOSURE

Lubricant compositions comprising a major amount of a lubricating base fluid and a minor amount of extreme pressure additives which contain either a methylene, monohalomethylene or dihalomethylene group between two moieties, selected from the group consisting of phosphono, dihydrocarblyphosphoryl, phenyl, substituted phenyl, keto, cyano, and carboxylate ester moieties. 15 20

#### REFERENCE TO RELATED APPLICATIONS

This application is a divisional of copending application Ser. No. 762,966, filed Sept. 26, 1968, and now U.S. Patent 3,579,449.

## BACKGROUND OF THE INVENTION

(1) Field of the invention

This invention relates to lubricant compositions which contain a lubricating base fluid and an additive to increase the load-bearing properties of the base fluid. These additives are generally referred to as extreme pressure additives. Ideally, the additives should improve the load-bearing properties of the base fluid without causing excessive corrosion problems, should be reasonably effective within their level of solubility or dispersability in the base fluid, and should be relatively easy to prepare.

## (2) Prior art

Halogen substituted compounds having phosphonate ester and carboxylate ester moieties are known as additives for lubricant compositions. See, for example, U.S. Patents 2,275,359; 2,599,761; 3,296,138; 2,225,366; 2,882,303-316; 2,824,839; 2,993,859; 2,722,515; 2,767-142; 2,882,228; and 2,848,475. However, the search has continued for effective extreme pressure lubricant additives and especially for such additives which are simple compounds that can be made economically and which do not cause excessive corrosion problems.

## THE INVENTION

This invention relates to lubricant compositions comprising (1) a major amount of a lubricating base fluid and (2) a minor amount sufficient to increase the load-bearing properties of said compositions of a compound having the formula:

YCX<sub>2</sub>Y

wherein each X is selected from the group consisting of hydrogen, chlorine, iodine and bromine atoms, each Y is selected from the group consisting of moieties having the following formulas

2

wherein each R is selected from the group consisting of alkyl, aryl, alkaryl, arylalkyl, alkenyl, haloalkyl, haloaryl, haloalkaryl, haloaralkyl, haloalkenyl and nitroaryl moieties containing from 1 to about 22 carbon atoms and each R<sup>1</sup> is selected from the group consisting of R, a halogen atom and a hydrogen atom, the above selections being made so that both X's can be hydrogen atoms only when both Y's are.

$$\begin{array}{c}
 \text{O} & \text{O}-\text{R} \\
 \parallel & \\
 \text{P} & \\
 | & \\
 \text{O} & \text{R}
 \end{array}$$

and that one X can be hydrogen only when each Y is selected from the group consisting of

$$\text{---P}(\text{O---R})_2 \text{---}, \text{---C}(=\text{O})\text{---O---R} \text{ and } \text{---C}\equiv\text{N}$$

### The lubricating base fluid

The extreme pressure additives of this invention will impart improved load-bearing characteristics to a wide variety of base fluids which are used for a variety of purposes. Broadly, the base fluid can be either a petroleum hydrocarbon, a fatty acid triglyceride, a synthetic fluid, an aqueous based fluid, or mixtures thereof. Petroleum hydrocarbons include mineral oil (including light solvents, neutral oils, heavy, bright and refined stocks, and asphaltic residual stocks), greases and waxes. The lubricating base fluid can also comprise suspensions of graphite in oils. Synthetic fluids include such disparate materials as polymerized olefins, organic carbonates, organic esters and/or ethers, polyglycols, silicones, modified organic materials (halogenated, phosphates, sulfurized, etc.) polymers e.g., alkylmethacrylate polymers and synthetic resins, e.g., resins formed by esterification of polyhydric alcohols with polycarboxylic acids. Examples of base fluids which can be used in the practice of this invention include those disclosed in U.S. Patent 2,599,761, especially columns 9-11; U.S. Patent 2,725,359, especially columns 2, and 7-8; U.S. Patent 2,767,142 especially column 4; U.S. Patent 2,882,228, especially columns 6-7; U.S. Patent 2,956,952, especially columns 3-5; U.S. Patent 2,993,859, especially columns 2-3; U.S. Patent 3,296,138, especially columns 6-10 and 12-20; and U.S. Patent 3,357,920, especially columns 5-7. Other suitable lubricating base fluids are disclosed in "Encyclopedia of Chemical Technology," Kirk-Othmer, second edition, volume 12, pages 557-616, especially pages 576-582, Interscience Publishers, 1967. More examples of metal working lubricant base fluids can be found in "Metal Working Lubricants," E. L. H. Bastian, first edition, McGraw-Hill Book Co., Inc. 1951. All of the above patents and books including the references referred to therein are incorporated herein by reference.

The finished lubricant composition containing the above lubricating base fluids and the extreme pressure additives disclosed hereinbefore and specifically described hereinafter, can be used for lubricants for automobiles, aircraft, etc. as gear and bearing lubricants; as industrial metal working lubricants, e.g., for metal cutting and extrusion of steel, aluminum, titanium and its alloys, etc. (cutting fluids, drawing fluids, drawing compounds, extrusion lubricants, forging lubricants, rolling oils, machine tool lubricants, and other similar lubricants); and as fluids for the transmission of power, e.g., in car transmissions or hydraulic systems.

## THE EXTREME PRESSURE ADDITIVE

The extreme pressure additives of this invention when added to the lubricating base fluids hereinbefore described

improve the load-bearing properties of said lubricating base fluids.

The extreme pressure additives of this invention are characterized by the presence of a methylene or halo (chloro, iodo, or bromo) substituted methylene group. This methylene group is attached to two other groups, each of which can be either a phosphono (phosphonate diester), carboxylate ester, keto, cyano, phosphoryl (e.g., dialkylphosphine oxide), phenyl or substituted phenyl group. These groups are essential to the good performance of the extreme pressure additives. These groups are also important in modifying the solubility of the extreme pressure additives in various lubricating base fluids. For example, those groups which contain alkyl groups can, by selecting the length of the alkyl groups, be modified to give various hydrophilic and hydrophobic properties to the extreme pressure additives. It will be noted that there is an optimum chain length for each extreme pressure additive for each lubricating base fluid.

The dihalo and monohalo extreme pressure additives of this invention can, in general, be prepared by reacting the non-halogenated compounds with the desired sodium hypohalite. See, e.g., O. T. Quimby et al., *J. Organometallic Chemistry*, 13, 199 (1968). The methylene diphosphonate esters can be prepared according to the teaching of U.S. Pat. 3,251,907. The dihalodicyanomethane extreme pressure additives can be prepared by reaction of the dicyanomethane with molecular halogen and subsequent decomposition of the alkali metal halide complex according to the teaching of Organic Synthesis, vol. 39, page 64, M. Tishler, Ed. and L. Ramberg and S. Widequist, *Arkiv Kemi, Mineral. Geol.*, 12A, No. 22 (1937). The dihalodiphenylmethane compounds are available commercially. All of the extreme pressure additives can be prepared by known or analogous methods. The iodo compounds are generally a mixture of mono- and diiodo compounds however.

Within the scope of the definition of the extreme pressure additives of this invention, there is a considerable variation in effectiveness with respect to extreme pressure properties and there is considerable variation with respect to other properties such as corrosivity, antiwear properties and, of course, solubility or dispersability. The non-halogenated methylenediphosphonate esters are the least corrosive of the additives. However, in general, they are also the least effective with respect to the extreme pressure properties. In general, the most effective extreme pressure additives are those which contain a dibromo-methylene group. However, they tend to be more corrosive than the other additives. Among the more effective extreme pressure additives are the dichloro-, diiodo- and dibromomethylenediphosphonates, the dibromomalonates, dibromomalononitrile, the tetrabromoglutarates, diphenyldichloromethane, dibenzoyldibromomethane, and the dibromo- and dichlorophosphonoacetates. The dichlorophosphonoacetates are equal to or slightly better than the dibromophosphonoacetates. This is a surprising reversal of the general trend in which the dibromo compounds are more effective than the dichloro compounds. In general, the alkyl groups should contain from 1 to about 6 carbon atoms. However, in the case of the malonates, it is preferred that the alkyl groups contain at least about 5 carbon atoms since the malonates containing alkyl groups with less than about 5 carbon atoms tend to be more corrosive.

Certain of the extreme pressure additives have a different primary activity. For example, when the alkyl groups contain from about 7 to about 22 carbon atoms, they are effective antiwear additives. This is especially true of the methylene- and halomethylenediphosphonate esters.

Although the additives which contain long chain alkyl groups are more effective as antiwear additives, they also are as effective as the shorter chain compounds, on a molar basis, as extreme pressure additives and the longer

chains are quite often more compatible with lubricants which are greases and waxes.

The iodo compounds, which are normally a mixture of mono- and diiodo compounds, are good additives for metal working lubricants, especially lubricants which are used in the working of titanium and titanium alloys.

In general there will be from 1% to about 20% of the additive, preferably from about 2% to about 10% in the lubricant composition.

10 Mixtures of extreme pressure additives can also be used. A synergistic mixture of tetraalkyl dichloromethylenediphosphonate and tricresyl phosphate, a well-known extreme pressure and anti-wear additive, is also preferred and is claimed in the application of Robert E Wann, Ser. No. 763,006, filed Sept. 26, 1968, and now abandoned.

15 Finished lubricant compositions containing the extreme pressure additives of this invention can also contain other known additives, e.g., antioxidants, corrosion inhibitors, metal deactivators, viscosity index improvers, dispersing materials, dyes, thickeners, etc. Examples of antioxidants include 2,6-ditertiarybutyl-4-methylphenol; 2,6-ditertiarybutyl phenol; 2,6-ditertiaryamyl-4-methylphenol; 2,6-diisopropyl-4-methylphenol; phenylnaphthylamine; phenylenediamine; and diphenylamine.

20 25 This invention can be better understood by reference to the following examples which should not be taken as limiting the scope of the invention.

Example I.—The following compositions were tested in a standard four ball tester for weld point (extreme pressure test) and wear scar (wear test). The weld point is defined as that pressure where the balls weld together in two successive runs of one minute under the indicated pressure. The wear scar is the average, based on three balls, of the average of both length and width of the scars when the balls are run under a 40 kg. load for one hour at 1200 r.p.m. and at a temperature of 130° F.

30 All of the indicated additives in the following table were added to a Kendall SAE 10, paraffin base, additive free oil (lubricating base fluid) at the indicated level.

| 40 | Composition                                                                        | Additive | Percent by weight | Weld point (kg.) | Wear scar (cm.) |
|----|------------------------------------------------------------------------------------|----------|-------------------|------------------|-----------------|
| 1  | — (base oil)                                                                       |          |                   | 130              | 0.82            |
| 2  | Sulfur, chlorine and lead naphthenate in fish oil (SCL)                            |          | 5                 | 240-260          | 0.76            |
| 3  | SCL                                                                                |          | 2                 | 216              | 0.68            |
| 4  | SCL                                                                                |          | 1                 | 180              | 0.70            |
| 5  | Tricresyl phosphate (TCP)                                                          |          | 5                 | 140              | 0.63            |
| 6  | Benzyl disulfide                                                                   |          | 5                 | 340              | 0.64            |
| 7  | Hexachlorethane                                                                    |          | 5                 | 210              | 0.64            |
| 8  | Tributyl phosphite                                                                 |          | 5                 | 200              | 0.70            |
| 9  | Trichloroacetic acid                                                               |          | 5                 | >70              | 1.01            |
| 10 | Randomly chlorinated paraffin                                                      |          | 5                 | 210              | 0.62            |
| 11 | Lead naphthenates                                                                  |          | 5                 | 230              | 0.72            |
| 12 | Molybdenum disulfide                                                               |          | 5                 | 140              | 0.80            |
| 13 | Tetrasopropyl dichloromethylenediphosphonate (IP <sub>4</sub> Cl <sub>2</sub> MDP) |          | 10                | 468              | —               |
| 14 | IP <sub>4</sub> Cl <sub>2</sub> MDP                                                |          | 5                 | 390              | 1.18            |
| 15 | IP <sub>4</sub> Br <sub>2</sub> MDP                                                |          | 2.5               | 360              | —               |
| 16 | IP <sub>4</sub> Cl <sub>2</sub> MDP                                                |          | 1                 | 270              | 0.94            |
| 17 | Tetraethyl dichloromethylenediphosphonate (Et <sub>4</sub> Cl <sub>2</sub> MDP)    |          | 5                 | 500              | 1.16            |
| 18 | Et <sub>4</sub> Cl <sub>2</sub> MDP                                                |          | 2.5               | 460              | 1.06            |
| 19 | Et <sub>4</sub> Cl <sub>2</sub> MDP                                                |          | 1                 | 270              | 0.94            |
| 20 | Tetramethyl dichloromethylenediphosphonate (Me <sub>4</sub> Cl <sub>2</sub> MDP)   |          | 5                 | 400              | —               |
| 21 | Tetrakis(decyldichloromethylenediphosphonate)                                      |          | 5                 | 210              | 0.49            |
| 22 | Tetrakis(stearyl)dichloromethylenediphosphonate                                    |          | 5                 | 160              | 0.345           |
| 23 | Tetraethyl dibromomethylenediphosphonate (Et <sub>4</sub> Br <sub>2</sub> MDP)     |          | 5                 | >800             | 1.19            |
| 24 | Et <sub>4</sub> Br <sub>2</sub> MDP                                                |          | 2.5               | 660              | 1.12            |
| 25 | Et <sub>4</sub> Br <sub>2</sub> MDP                                                |          | 1                 | 250              | 0.60            |
| 26 | Tetrasopropyl dibromomethylenediphosphonate (IP <sub>4</sub> Br <sub>2</sub> MDP)  |          | 5                 | 400              | 1.12            |
| 27 | Tetrasopropyl monobromomethylenediphosphonate                                      |          | 5                 | 270              | 1.14            |
| 28 | Tetrasopropyl monochloromethylenediphosphonate                                     |          | 5                 | 280              | 1.07            |
| 29 | Tetrasopropyl methylenediphosphonate                                               |          | 5                 | 260              | 1.02            |
| 30 | Tetraethyl methylenediphosphonate                                                  |          | 5                 | 190              | —               |
| 31 | Tetrakis(stearyl)methylenediphosphonate (C <sub>18</sub> MDP)                      |          | 5                 | 140              | 0.375           |
| 32 | Diethyl trichloromethylphosphonate <sup>1</sup>                                    |          | 5                 | >800             | 0.96            |

| Composition | Additive                                                                  | Percent by weight | Weld point (kg.) | Wear scar (cm.) |
|-------------|---------------------------------------------------------------------------|-------------------|------------------|-----------------|
| 33          | iPr <sub>4</sub> Cl <sub>2</sub> MDP + C <sub>18</sub> MDP (1:1)          | 10                | 360              | 0.78            |
| 34          | Triethyl dichlorophosphonoacetate                                         | 5                 | 660              | 0.95            |
| 35          | Triethyl dibromophosphonoacetate                                          | 5                 | 600              | 2.41            |
| 36          | Diphenylmethylene dichloride                                              | 5                 | 400              | 1.42            |
| 37          | Diethyl dibromomalonate <sup>1</sup>                                      | 5                 | >800             | 0.68            |
| 38          | Diethyl dichloromalonate                                                  | 5                 | 250              | 0.71            |
| 39          | Diethyl malonate                                                          | 5                 | 130              | 0.76            |
| 40          | Di(isopentyl) dibromomalonate (nC <sub>6</sub> Br <sub>2</sub> Mal.)      | 5                 | >800             | -----           |
| 41          | do                                                                        | 3                 | 500              | -----           |
| 42          | do                                                                        | 2                 | 380              | -----           |
| 43          | do                                                                        | 1                 | 280              | -----           |
| 44          | Di(isopentyl) dibromomalonate (C <sub>6</sub> Br <sub>2</sub> Mal.)       | 5                 | >800             | -----           |
| 45          | do                                                                        | 3                 | 380              | -----           |
| 46          | do                                                                        | 2                 | 320              | -----           |
| 47          | do                                                                        | 1                 | 280              | -----           |
| 48          | Diethyl dibromomalonate (Et Br <sub>2</sub> Mal.) <sup>1</sup>            | 5                 | >800             | -----           |
| 49          | do                                                                        | 3                 | >800             | -----           |
| 50          | do                                                                        | 2                 | 780              | -----           |
| 51          | do                                                                        | 1                 | 500              | -----           |
| 52          | Tris(decyl) dibromophosphonoacetate (C <sub>10</sub> Br <sub>2</sub> PA). | 5                 | 240              | -----           |
| 53          | Triethyl chlorophosphonoacetate (Et Cl PA).                               | 5                 | 260              | -----           |
| 54          | Triethyl phosphonacetate (Et PA).                                         | 5                 | 120              | -----           |
| 55          | Tetrakis(decyl) methylene-diphosphonate (C <sub>10</sub> MDP).            | 5                 | 140              | -----           |
| 56          | Tetrabenzyl methylene-diphosphonate (Benzyl MDP).                         | 5                 | 120              | -----           |
| 57          | Tetrabenzyl dichloromethylene-diphosphonate (Benzyl Cl <sub>2</sub> MDP). | 5                 | 220              | -----           |
| 58          | Tetraisopropyl diiodomethylene-diphosphonate.                             | 5                 | 500              | -----           |
| 59          | Dimethyl 3-keto-2,2,4,4-tetrabromogluarate                                | 5                 | >800             | -----           |
| 60          | Dibromomalononitrile                                                      | 5                 | >800             | -----           |
| 61          | Dibenzoyl dibromomethane                                                  | 5                 | 560              | -----           |

<sup>1</sup> Very corrosive.

Compositions 2-12 and 32 demonstrate the effectiveness of certain representative prior art extreme pressure additives. It should be noted that, with the exception of the trichloroacetic acid and the diethyl trichloromethylphosphonate, the weld points are well under 400 kg. at an additive level of about 5%. The trichloroacetic acid and trichloromethylphosphonate, however, are quite corrosive.

Compositions 13-19, 23-25, and 40-51 show the effect of varying the level of six representative extreme pressure additives of this invention. At a level of only about 1% they are still better than most conventional additives at a level of 5%.

Compositions 20-22 shows the effect of changing the length of the alkyl chain. The longer alkyl chains merely dilute the extreme pressure additive effect, since on a molar basis the improvements of the additives of compositions 20-22 are about the same. There is a major difference however in anti-wear properties since the tetrakis(decyl) and tetrakis(stearyl) additives provide a major improvement as demonstrated by the wear scar. The tetramethyl additive does not help the antiwear properties of the base fluid.

A comparison of Compositions 17 and 23; 14 and 26; and 37 and 38 shows that, in general, the dibromo additives are more effective than the dichloro additives. This is especially true with the malonates. Similarly, a comparison of Compositions 14, 26 and 58 shows that for the particular tetraisopropyl methylenediphosphonate additives the diiodo derivative is better than the dibromo derivative which is better than the dichloro derivative. However, the ranking of the diiodo compound is undoubtedly affected by the fact it contained a substantial amount of monoiodomethylenediphosphonate.

A comparison of Compositions 26, 27 and 29; 14, 28 and 29; 17 and 30; 21 and 55; 23 and 30; 37 and 39; 38 and 39; and 34, 53 and 54 shows the effect of going from a nonhalogenated to a monohalogenated to a dihalogenated extreme pressure additive having the same basic structure. In general the nonhalogenated compounds are not effective extreme pressure additives. However,

surprisingly, the methylenediphosphonate esters have substantial extreme pressure activity. The monohalogenated compounds in general are not much better than the nonhalogenated compounds as extreme pressure additives and it is only with the dihalogenated compounds that the best extreme pressure activity is achieved. It is surprising that the change from monohalogenated to dihalogenated compounds would give such a tremendous increase in extreme pressure activity.

10 As compositions 22 and 31 show the antiwear properties are affected only slightly by the presence or absence of the halogen atoms on a compound. Also, in composition 33 a mixture of a extreme pressure additive

(iPr<sub>4</sub>Cl<sub>2</sub>MDP)

15 and an anti-wear additive (C<sub>18</sub>MDP) gives both good extreme pressure activity and anti-wear activity.

A comparison of the above composition shows that the dichloro- and dibromomethylenediphosphonates, the dichloro- and dibromophosphonoacetates, the dibromomalonates, the dibromomalononitrile, and the tetrabromoglutarates give the best extreme pressure activity. The dichloromalononitrile and the tetrachloroglutarates are also good. The diiodomethylenediphosphonates, dibenzoyldibromomethane, and the diphenylmethylene dichloride are also very good extreme pressure additives. These compounds, in general, will give a weld point in the four ball test of at least about 400 kg. when used at the 5% level in this base fluid.

20 30 The dimethyl 3-keto-2,2,4,4-tetrabromogluarate (Composition 59) is a difunctional dibromomethylene compound which shows that more than one YCX<sub>2</sub>Y group can be present in a molecule of the extreme pressure additives of this invention.

35 Tetrabenzyl methylenediphosphonates are not very soluble in the base fluid of this example and accordingly are not as effective in this fluid as some of the other extreme pressure additives.

The diethyl dibromomalonates, e.g., compositions 37 40 and 48-51 are extremely corrosive. The dipentyl and diisopentyl esters of the dichloro- and dibromomalonates, e.g., compositions 40-47 are not corrosive.

In the following compositions, a comparison has been made between a base oil containing only the additives of 45 this invention (Kendall base oil) and an oil containing a complete additive package including a corrosion inhibitor (Havoline). The corrosion inhibitor apparently has an adverse effect upon the extreme pressure activity, but the extreme pressure activity is still very good and the corrosiveness is minimized. Tetraisopropyl dichloromethylenediphosphonate is not as corrosive to steel as the other three additives and is included for comparison.

| Additive                                                                                  | Base oil    | Concentration of the additive (weight percent) |            |
|-------------------------------------------------------------------------------------------|-------------|------------------------------------------------|------------|
|                                                                                           |             | Weld point                                     | Weld point |
| Tetraethyl dibromomethylene-diphosphonate (Et <sub>4</sub> Br <sub>2</sub> MDP).          | Kendall...  | 5                                              | >800       |
| Do                                                                                        | Havoline... | 5                                              | 425        |
| 60 Tetraisopropyl dibromomethylene-diphosphonate (iPr <sub>4</sub> Br <sub>2</sub> MDP).  | Kendall...  | 5                                              | 400        |
| Do                                                                                        | Havoline... | 5                                              | 320        |
| Tetraethyl dichloromethylene-diphosphonate (Et <sub>4</sub> Cl <sub>2</sub> MDP).         | Kendall...  | 5                                              | 500        |
| Do                                                                                        | Havoline... | 5                                              | 340        |
| 65 Tetraisopropyl dichloromethylene-diphosphonate (iPr <sub>4</sub> Cl <sub>2</sub> MDP). | Kendall...  | 5                                              | 360-440    |
| Do                                                                                        | Havoline... | 5                                              | 300        |

In the following compositions the base fluid was water.

| Additive                            | Percent by weight | Weld point (kg.) |
|-------------------------------------|-------------------|------------------|
| Me <sub>4</sub> Cl <sub>2</sub> MDP | 5                 | 50<br>130        |

Example II.—The following compositions are excellent lubricants having better extreme pressure characteristics than the lubricating base fluid.

| Extreme pressure additive                                                                                                                 | Lubricating base fluid                                                                                                                                                                                 | Additive, percent by weight |
|-------------------------------------------------------------------------------------------------------------------------------------------|--------------------------------------------------------------------------------------------------------------------------------------------------------------------------------------------------------|-----------------------------|
| 1. Dibromodicyanomethane                                                                                                                  | Allyl laurate                                                                                                                                                                                          | 3.5                         |
| 2. Dichlorodicyanomethane                                                                                                                 | Propyl propionate                                                                                                                                                                                      | 4.0                         |
| 3. Dibromocyan (diethylphosphono)methane                                                                                                  | Trioctyl phosphate                                                                                                                                                                                     | 5.0                         |
| 4. Dibromo(phenylmethyl)(dimethylphosphoryl)methane                                                                                       | Diethyl carbonate                                                                                                                                                                                      | 5.0                         |
| 5. Dichloro(disopropylphosphono)decanoylmethane                                                                                           | Isopropyl myristate                                                                                                                                                                                    | 4.0                         |
| 6. Ethyl dichlorocyanacetate                                                                                                              | Stearyl acetate                                                                                                                                                                                        | 5.0                         |
| 7. Dibromocyanooctanoylmethane                                                                                                            | Diethyl ether of ethylene glycol                                                                                                                                                                       | 3.0                         |
| 8. Dicloro(butylmethylphosphoryl)cyanomethane                                                                                             | Glycerol                                                                                                                                                                                               | 3.0                         |
| 9. Dichlorodiphosphorylmethane                                                                                                            | Naphthalene                                                                                                                                                                                            | 4.0                         |
| 10. Dibromo(methylphenyl)(dodecylphenyl)methane                                                                                           | Petrolatum                                                                                                                                                                                             | 5.0                         |
| 11. Bromochloro(decylphenyl)(diethylphenyl)methane                                                                                        | Paraffin wax                                                                                                                                                                                           | 5.0                         |
| 12. Dichloro(biphenyl)(naphthyl)methane                                                                                                   | 1:1 mixture of naphthalene and xylene                                                                                                                                                                  | 5.0                         |
| 13. Dibromo(chlorophenyl)(3,4-dinitrophenyl)methane                                                                                       | Diethylphthalate                                                                                                                                                                                       | 4.0                         |
| 14. Dibromobis(butylethylphosphoryl)methane                                                                                               | Propylene glycol                                                                                                                                                                                       | 3.0                         |
| 15. Dibromo di(ethylbutylphosphoryl)methane                                                                                               | Methyl ethyl ketone                                                                                                                                                                                    | 4.0                         |
| 16. Chlorobromo(tetrachlorostearylmethylphosphonio)-tetra-fluorostearylmethylphosphonio)methane                                           | Carnauba wax                                                                                                                                                                                           | 5                           |
| 17. Dichloro(dinitrophenyl)(methyl dichloroacetylphosphonio) methane                                                                      | Tallow                                                                                                                                                                                                 | 5                           |
| 18. Ethyl dibromo(dimethylphosphonio)acetate                                                                                              | Stearyl alcohol                                                                                                                                                                                        | 5                           |
| 19. Di(2-iodoacetyl) dibromomethane                                                                                                       | 20% emulsion of tallow in water                                                                                                                                                                        | 10                          |
| 20. Di(acetyl)dichloromethane                                                                                                             | Octyl tripropylene glycol ether                                                                                                                                                                        | 5                           |
| 21. Dipentyl monochloromalonate                                                                                                           | Mineral oil S.A.E. 10                                                                                                                                                                                  | 5                           |
| 22. Di(methylbenzoyl)dibromomethane                                                                                                       | Rosin                                                                                                                                                                                                  | 4                           |
| 23. Bromostearyl bromomethyl bromomalonate                                                                                                | 1:1 phenol-formaldehyde resin (M.W. 1,200)                                                                                                                                                             |                             |
| 24. Stearyl behenyl dichloromalonate                                                                                                      | Grease (lubricating oil thickened with soap)                                                                                                                                                           | 5                           |
| 25. Dodecanyl bromobenzyl dibromomalonate                                                                                                 | Isopropyl laurate                                                                                                                                                                                      | 6                           |
| 26. Iodobenzoyl (diidoethylphosphono)dichloromethane                                                                                      | 1:1 mixture of isopropyl and alcohol                                                                                                                                                                   | 5                           |
| 27. Biphenylaphthalyl dibromomethane                                                                                                      | Kerosene                                                                                                                                                                                               | 4                           |
| 28. Dihexyl chloromalonate                                                                                                                | Turbine oil                                                                                                                                                                                            | 5                           |
| 29. Iodomethyl iodobenzyl dibromomalonate                                                                                                 | 40% soybean oil in water emulsion                                                                                                                                                                      | 0                           |
| 30. Di(2-ethylhexyl) dibromomalonate                                                                                                      | Di(2-ethylhexyl) sebacate                                                                                                                                                                              | 5                           |
| 31. Bromodicyanomethane                                                                                                                   | 10% suspension of graphite in mineral oil SAE 10                                                                                                                                                       | 8                           |
| 32. Chlorodicyanomethane                                                                                                                  | Polyethylene glycol (M.W. 1,800)                                                                                                                                                                       | 5                           |
| 33. Ethyl chlorocyanacetate                                                                                                               | Polypropylene glycol (M.W. 2,200)                                                                                                                                                                      | 4                           |
| 34. Chlorocyan (disopropylphosphono)methane                                                                                               | Octylether of polyethylene glycol (M.W. 4,000)                                                                                                                                                         | 5                           |
| 35. Bromocyan (cetyltrimethylphosphoryl)methane                                                                                           | Di-2-ethylhexanate of 1:1 ethylene glycol propylene glycol (M.W. 6,000)                                                                                                                                | 7                           |
| 36. Octadecenyl (dibromobutyl octadecenylphosphoryl)acetate                                                                               | Stearyl stearate                                                                                                                                                                                       | 10                          |
| 37. Dichloro(dimethylphosphonio)(dimethylphosphono)methane                                                                                | 20% cottonseed oil in water emulsion with 5% alkyl (C <sub>11</sub> -15) poly ethoxylate (9 moles) emulsifier                                                                                          | 10                          |
| 38. Dibromodi (3,4-difluorophenyl)methane                                                                                                 | Winterized and hardened (I.V. 8) soybean oil                                                                                                                                                           | 5                           |
| 39. Tri benzyl bromochlorophosphonate                                                                                                     | Naphthenic hydrocarbon oil                                                                                                                                                                             | 5                           |
| 40. Tetra (tetrafluorostearyl) dibromomethylene diphosphonate                                                                             | Fluorinated polypropylene (M.W. 1,000)                                                                                                                                                                 | 10                          |
| 41. Dichloro di(3,4,5-trichlorophenyl)methane                                                                                             | Di-n-butylphthalate                                                                                                                                                                                    | 4                           |
| 42. Dibromoacetyl(propionyl)methane                                                                                                       | 1:1 mixture of di-(2-butoxyethyl) azelate and di(methylcyclohexyl)adipate                                                                                                                              | 4                           |
| 43. 3-bromopropyl dibromo(4,5-dichlorodecanoyl) acetate                                                                                   | The condensation product of propylene glycol, ethylene glycol, phthalic acid and sebacic acid in a 3:2:1:1 ratio (M.W. 2,000). The C <sub>8</sub> -C <sub>10</sub> oxo alcohol esters of phthalic acid | 6                           |
| 44. Dibromo hexanoyl (butylpropylphosphono)methane                                                                                        | Butyl ether of polyethylene glycol (M.W. 1,000)                                                                                                                                                        | 5                           |
| 45. Dichlorobenzoyl (ditolylphosphono)methane                                                                                             | A 3:1 mixture of butyl ether of polypropylene glycol (M.W. 1,600) and diisooctyl adipate                                                                                                               | 6                           |
| 46. A 5:2 mixture of tri(decylphenyl) dichlorophosphono acetate and N-phenyl-alpha-naphthylamine                                          | Diethylpentadecandicarboxylate                                                                                                                                                                         | 6                           |
| 47. Bromochloro(decylphenyl)-decanoylmethane                                                                                              | Dimethylsilicone polymer (M.W. 3,000)                                                                                                                                                                  | 5                           |
| 48. Dimethylidibutyl methylene diphosphonate                                                                                              | Mineral oil SAE 30                                                                                                                                                                                     | 6                           |
| 49. Ethyldecyhexyl dibromophosphonate                                                                                                     | Petroleum wax                                                                                                                                                                                          | 10                          |
| 50. Dibromo[(2,3-dichloroethylphenyl) (3,4-difluorobenzyl)phosphono] [(5,6-dibromo-2-decenoyl) methylphosphonon]methane                   | Kendall base oil (SAE 10)                                                                                                                                                                              | 5                           |
| 51. 1:1 mixture of bis(2-ethylhexyl) dibromo-malonate and tetra-methylidichloromethylenediphosphonate                                     | do                                                                                                                                                                                                     | 5                           |
| 52. 1:1:1 mixture of tetraisopropyl dibromomethylenediphosphonate, triethyl dichlorophosphonate, and bis (2-ethylhexyl) di-chloromalonate | Kendall base oil (SAE 20)                                                                                                                                                                              | 5                           |
| 53. Diacetyl dibromomethane                                                                                                               | Cotton seed oil                                                                                                                                                                                        | 10                          |
| 54. Dibenzoyldifluoromethane                                                                                                              | Bis(2-ethylhexyl) sebacate                                                                                                                                                                             | 4                           |
| 55. Bis(2-chloroethyl) dichloromalonate                                                                                                   | Kendall base oil (SAE 10)                                                                                                                                                                              | 5                           |
| 56. Dihexyl dibromomalonate                                                                                                               | Bis(2-ethylhexyl) adipate                                                                                                                                                                              | 6                           |
| 57. Dibromomalononitrile                                                                                                                  | Decyl decanoate                                                                                                                                                                                        | 5                           |
| 58. n-Decyl dibromocyanacetate                                                                                                            | Naphthalene                                                                                                                                                                                            | 3                           |
| 59. Tetrabenzyl dichloromethylenediphosphonate                                                                                            | Soybean oil                                                                                                                                                                                            | 8                           |
| 60. Tris(p-nitrobenzyl) diisopropylphosphonate                                                                                            | Paraffin                                                                                                                                                                                               | 4                           |
| 61. Bis(bis(fluoromethyl)phosphoryl) dichloromethane                                                                                      | Tripropylene glycol didecanate                                                                                                                                                                         | 5                           |
| 62. Bis(2,4-dichlorobenzoyl) dibromomethane                                                                                               | Stearyl stearate                                                                                                                                                                                       | 8                           |
| 63. Dioleyl dibromomalonate                                                                                                               | Stearyl benzoate                                                                                                                                                                                       | 10                          |
| 64. Bis(p-dodecylbenzoyl) dichloromethane                                                                                                 | 10% suspension of graphite in kerosene                                                                                                                                                                 | 10                          |
| 65. Bromodomalononitrile                                                                                                                  | Polypropylene glycol (M.W. 600)                                                                                                                                                                        | 6                           |
| 66. Tetraisopropyl bromodomalonenediphosphonate                                                                                           | Polyethylene glycol (M.W. 900)                                                                                                                                                                         | 5                           |
| 67. Dipentyl cyanodibromomethylphosphonate                                                                                                | Petroleum wax                                                                                                                                                                                          | 6                           |
| 68. Tetrakis(2,3-dibromopropyl) dibromomethylenediphosphonate                                                                             | do                                                                                                                                                                                                     | 15                          |
| 69. Bis(9,10-dichlorostearyl) bromomalonate                                                                                               | 1,2-trichloroethane                                                                                                                                                                                    | 6                           |
| 70. Tris(2,2,2-trichloroethyl) dichlorophosphonate                                                                                        | Kerosene                                                                                                                                                                                               | 3                           |
| 71. Bromodicyanomethane                                                                                                                   | 20% emulsion of tallow in water with 5% coconut alkyl poly-ethoxylate (15 moles ethylene oxide) emulsifier                                                                                             | 6                           |
| 72. Tetraethyl diiodomethylenediphosphonate                                                                                               | Kendall base oil (SAE 30)                                                                                                                                                                              | 5                           |
| 73. Pentyldichlorocyanacetate                                                                                                             | Kendall base oil (SAE 10)                                                                                                                                                                              | 5                           |
| 74. Dibromodiphenylmethane                                                                                                                | Winterized and slightly hardened (I.V. 10) soybean oil                                                                                                                                                 | 8                           |
| 75. Bis(p-nitrophenyl) diiodomethane                                                                                                      | Tallow                                                                                                                                                                                                 | 5                           |
| 76. Cyanodibromophenylmethane                                                                                                             | Methyl stearate                                                                                                                                                                                        | 8                           |
| 77. Dicyclohexyl bromomalonate                                                                                                            | Fluorinated polypropylene (M.W. 2,000)                                                                                                                                                                 | 8                           |
| 78. Ethyl (perfluorophenyl) dibromoacetate                                                                                                | Polyvinyl chloride (M.W. 800)                                                                                                                                                                          | 5                           |
| 79. Tetramethyl dichloromethylenediphosphonate                                                                                            | Bis(2-ethylhexyl) sebacate                                                                                                                                                                             | 6                           |
| 80. Bis(2-ethylhexyl) dibromomalonate                                                                                                     | Bis(2-ethylhexyl) adipate                                                                                                                                                                              | 5                           |
| 81. Bis(2-methylbutyl) bromomalonate                                                                                                      | Propylene glycol disterate                                                                                                                                                                             | 4                           |
| 82. Bis(diethylphosphoryl) dichloromethane                                                                                                | Kendall base oil (SAE 20)                                                                                                                                                                              | 5                           |
| 83. Dimethyl 3-keto-2,2,4-tetrabromoglutarate                                                                                             | Tetrapropylene glycol dioctyl ether                                                                                                                                                                    | 8                           |
| 84. Benzoyl trifluoroacetyl dibromomethane                                                                                                | Kendall base oil (SAE 20)                                                                                                                                                                              | 5                           |
| 85. Pentyldichloroacetyl dichloroacetate                                                                                                  | Paraffin                                                                                                                                                                                               | 9                           |
| 86. Pentachlorobenzoylvinylodibromomethane                                                                                                | Grease                                                                                                                                                                                                 | 12                          |
| 87. (Diphenylphosphoryl) propionylchloromethane                                                                                           | Naphthalene                                                                                                                                                                                            | 8                           |
| 88. Diphenylphosphorylcyanodimethane                                                                                                      |                                                                                                                                                                                                        |                             |

TABLE—Continued

| Extreme pressure additive                               | Lubricating base fluid                                                                          | Additive, percent by weight |
|---------------------------------------------------------|-------------------------------------------------------------------------------------------------|-----------------------------|
| 89. Dipropyl phenyldichloromethylphosphonate            | Diethyl phthalate                                                                               | 5                           |
| 90. Tetrakis(decyl) bromochloromethylenediphosphonate   | Kendall base oil (SAE 30)                                                                       | 5                           |
| 91. Tetrakis(stearyl) bromochloromethylenediphosphonate | Tallow                                                                                          | 5                           |
| 92. Bis(behenyl) dibromomalonate                        | Behenyl behenate                                                                                | 20                          |
| 93. Stearyl bromiodocyanacetate                         | Stearyl acetate                                                                                 | 10                          |
| 94. Divinyl cyanodichloromethylphosphonate              | Kendall base oil (SAE 10)                                                                       | 5                           |
| 95. Dichloromalononitrile                               | 20% soybean oil in water emulsion; 5% tallow fatty alcohol polyethoxylate (45 moles) emulsifier | 5                           |
| 96. Tetraethyl dibromomethylenediphosphonate            | Pentapropylene glycol diundecanoate                                                             | 5                           |
| 97. Tetraethyl dichloromethylenediphosphonate           | Tripropylene glycol didecanoate                                                                 | 5                           |
| 98. Tetraisopropyl dibromomethylenediphosphonate        | Hayoline oil                                                                                    | 5                           |
| 99. Tetraisopropyl dichloromethylenediphosphonate       | Bis(2-ethylhexyl) adipate                                                                       | 5                           |
| 100. Tetraisopropyl methylenediphosphonate              | Tetrapropylene glycol dodecanoate                                                               | 5                           |
| 101. Tetraisopropyl bromomethylenediphosphonate         | Kendall base oil (SAE 10)                                                                       | 5                           |
| 102. Diethyl dibromomalonate                            | do                                                                                              | 5                           |
| 103. Bis(benzoyl) dibromomethane                        | Cotton seed oil                                                                                 | 5                           |
| 104. Dipentyl diiodomalonate                            | Soybean oil                                                                                     | 15                          |
| 105. Pentyl 3-keto-2,2-dibromobutyrate                  | Kendall base oil (SAE 20)                                                                       | 5                           |

Example III.—In the following test the following additives were added to the Kendall base oil of Example I to give an additive level of about 5% by weight of the composition and coupons of the indicated metals were exposed to the oil/additive composition in air at a temperature of about 275° F. for 100 hours at the rate of 5 liters per hour. The numbers given are the weight changes in milligrams per square centimeter of surface area.

|              | iPr <sub>4</sub> Cl <sub>2</sub> MDP | iPr <sub>4</sub> Br <sub>2</sub> MDP |
|--------------|--------------------------------------|--------------------------------------|
| Magnesium    | 0.428                                | 0.210                                |
| Aluminum     | 0.038                                | 0.045                                |
| Steel (soft) | 0.046                                | 0.173                                |
| Copper       | 1.875                                | 0.195                                |
| Silver       | 0.053                                | 0.555                                |

Example IV.—The following table compares the base oil of Example I with compositions containing the indicated amounts of the indicated additives in a four ball tester, a Timken tester, and a Falex tester. All three tests should be used to determine if the extreme pressure additive has wide utility. The representative additives of this invention are all clearly superior to the commercially available additives.

|                            | Base oil | 5% TCP | 5% SCL | 5% iPr <sub>4</sub> Cl <sub>2</sub> MDP | 5% iPr <sub>4</sub> Cl <sub>2</sub> MDP | 2.5% Et <sub>4</sub> Cl <sub>2</sub> MDP | 5% Et <sub>4</sub> Cl <sub>2</sub> MDP | 2.5% Et <sub>4</sub> Cl <sub>2</sub> MDP | 2.5% iPr <sub>4</sub> Br <sub>2</sub> MDP | 2.5% iPr <sub>4</sub> Br <sub>2</sub> MDP | 2.5% Et <sub>4</sub> Br <sub>2</sub> MDP |
|----------------------------|----------|--------|--------|-----------------------------------------|-----------------------------------------|------------------------------------------|----------------------------------------|------------------------------------------|-------------------------------------------|-------------------------------------------|------------------------------------------|
| Four Ball:                 |          |        |        |                                         |                                         |                                          |                                        |                                          |                                           |                                           |                                          |
| Load wear index            | 18.4     | 26.6   | 25.1   | 53.6                                    | 33.6                                    | 72.9                                     | 62.0                                   | 50.3                                     | 105.9                                     |                                           |                                          |
| Weld point (kg.)           | 112      | 112    | 224    | 316                                     | 251                                     | 501                                      | 355                                    | 251                                      | 562                                       |                                           |                                          |
| Timken: (Beam load in lb.) | 3        | 12     | 18     |                                         | 55                                      |                                          | 65                                     | 75                                       | 65                                        |                                           |                                          |
| Falex:                     |          |        |        |                                         |                                         |                                          |                                        |                                          |                                           |                                           |                                          |
| (Load in lb.)              | 500      | 1,250  | 1,000  |                                         | 14,500                                  |                                          | 14,500                                 | 14,500                                   | 14,500                                    |                                           |                                          |
| (Torque in lb.-in.)        |          |        |        |                                         | (50)                                    |                                          | (66)                                   | (64)                                     | (60)                                      |                                           |                                          |

<sup>1</sup> Capacity of instrument.

NOTE.—All parts, percentages, and ratios herein are by weight unless otherwise specified. The four ball results in Example IV were obtained on a different testing machine than the results in the other examples which caused the discrepancy.

#### References Cited

#### UNITED STATES PATENTS

3,181,992 5/1965 Michalski et al. 106—15

#### FOREIGN PATENTS

785,198 10/1957 Great Britain.

DANIEL E. WYMAN, Primary Examiner

W. H. CANNON, Assistant Examiner

What is claimed is:

1. A lubricant composition comprising  
(1) a major amount of a lubricating base fluid and  
(2) a minor amount sufficient to increase the load-bearing properties of said compositions of a compound have the formula:



wherein one X is selected from the group consisting of hydrogen, atoms, the other X is bromine and wherein each R is selected from the group consisting of alkyl, aryl, alkaryl, aralkyl, alkenyl, haloalkyl, haloaryl, haloalkaryl, haloaralkyl, haloalkenyl and nitroaryl moieties containing from 1 to about 22 carbon atoms.

2. The composition of claim 1 wherein component (2) is a dibromomalonate.

3. The composition of claim 1 wherein each R is an alkyl group containing from about 5 to about 22 carbon atoms.

4. The composition of claim 1 wherein there is from about 1% to about 20% of component (2).

5. The composition of claim 1 wherein there is from about 2% to about 10% of component (2).

6. The composition of claim 2 wherein each R is an alkyl group containing from about 5 to about 22 carbon atoms.

UNITED STATES PATENT OFFICE  
CERTIFICATE OF CORRECTION

Patent No. 3,691,077

Dated September 12, 1972

Inventor(s) Robert Earl Wann, Denzel Allan Nicholson & Ted Joe Logan

It is certified that error appears in the above-identified patent  
and that said Letters Patent are hereby corrected as shown below:

Page 1, Column 1, in the heading after Cincinnati, Ohio, add  
--- Assignors to the Procter & Gamble Company, Cincinnati, Ohio,  
a corporation of Ohio ---.

Col. 1, line 19, after "moieties" and before "selected" delete  
",".

Col. 1, line 45, delete "2,275,359" and insert therefore ---  
2,725,359 ---.

Col. 2, line 2, delete "arylalkyl" and insert therefore ---  
aralkyl ---.

Col. 2, line 35, delete "phosphates" and insert therefore ---  
phosphated ---.

Col. 3, line 26, delete "teaching" and insert therefore ---  
teachings ---.

Col. 4, line 47, (In the Table under Weld Point (kg.)) number 9  
delete "<70" and insert therefore --- <700 ---.

Col. 6, line 72, delete second occurrence of "point".

Col. 8, Example 29 under "additive percent by weight" delete "0"  
and insert therefore --- 10 ---.

Col. 10, line 27, after the first comma and before "atoms" insert  
--- and bromine ---.

Col. 10, line 27, after "bromine" and before "and" insert  
---, ---.

Signed and sealed this 19th day of November 1974.

(SEAL)  
Attest:

McCOY M. GIBSON JR.  
Attesting Officer

C. MARSHALL DANN  
Commissioner of Patents